

Sept. 24, 1968

W. H. CHANG

3,403,022

CHROMIUM BASE ALLOY

Filed Oct. 14, 1965



INVENTOR  
WINSTON H. CHANG  
BY  
*Lee H. Chang*

ATTORNEY —

1

3,403,022

## CHROMIUM BASE ALLOY

Winston H. Chang, Cincinnati, Ohio, assignor to General Electric Company, a corporation of New York  
Filed Oct. 14, 1965, Ser. No. 495,998  
2 Claims. (Cl. 75—176)

This invention relates to a chromium base alloy and, more particularly, to a chromium base alloy of improved strength particularly in sheet form.

Advances in gas turbine technology for power producing apparatus has identified a need for improved materials useful at elevated temperatures. At 1800° F. and above, some of the currently used iron, nickel or cobalt base superalloys have been found to have limitations for certain applications. Therefore, improvement of the refractory metals such as molybdenum, columbium and chromium has been the subject of wide effort. Of these materials, chromium is attractive because of its inherently better oxidation resistance compared with the other refractory metals.

It is a principal object of the present invention to provide a chromium base alloy of improved high temperature strength and having ductility sufficient to allow easy reduction from cast to sheet form.

Another object is to provide an improved chromium base alloy having improved high temperature strength as well as a recrystallization temperature sufficiently high to further take advantage of work hardening and inhibit embrittlement of the alloy.

These and other objects and advantages will be more fully understood from the following detailed description and examples which are meant to be exemplary of rather than any limitation on the scope of the present invention.

The drawing is a graphical comparison of tensile properties between a known sheet alloy and that of this invention.

It has been recognized that a chromium base alloy of improved strength can be provided by the addition of a particular amount of columbium, in the presence of carbon in certain proportions to control a fine dispersion of columbium carbide. This dispersion within the range of this invention strengthens chromium both in the cast as well as in the wrought condition yet the amount of carbon is controlled to avoid formation of the embrittling chromium carbide phase.

In one form, the alloy of the present invention consists essentially of, by weight, 0.05—0.15% C; 0.5—1.5% Cb; 0.05—0.2% Y; 0.05—0.2% Th; up to 0.2% Zr; with the balance essentially chromium and incidental impurities.

Elements of the Periodic Table of Elements in Group IV-A, of which zirconium is typical, and Group V-A, of which columbium is typical, have been broadly specified for addition to some of the refractory metals, particularly columbium and molybdenum. However, in the case of chromium as a base, it has been recognized that all types of carbide dispersions do not play the same role in strengthening.

The relationship of alloying additions such as the Group IV-A and Group V-A metals along with carbon in chromium base alloys is particularly significant. The flow and fracture behavior of chromium is profoundly affected by interstitials. The arrangements, size and type of carbide has been found to affect strength, ductility and air oxidation in different ways. The influence of processing and heat treatment in controlling these kinds of mechanisms and hence the properties is significantly important in chromium base alloys. For example, in the presence of about 0.1 weight percent carbon in a chromium base, the element zirconium will form a carbide precipitate significantly different from that formed through the addition

2

of columbium. The zirconium carbide, because of its relatively low solubility in chromium, forms in the as-cast condition a carbide network in the grain boundaries. Columbium has a greater solubility in chromium than does zirconium. Hence in the presence of carbon, columbium will precipitate as a fine rather than coarse dispersion of columbium carbide throughout the matrix as well as in the grain boundary of the chromium base structure. Thus the columbium addition will provide greater strengthening to the alloy because of the formation of a fine precipitate different in kind than that of zirconium. Furthermore, it has been found that whereas chromium base alloys strengthened with columbium carbide tend to be brittle in the recrystallized condition, in the stress relief conditions they have significantly improved strength. By maintaining the addition of columbium and its relationship to carbon within the range of 0.5—1.5 weight percent columbium and 0.05—0.15 weight percent carbon, the recrystallization temperature can be maintained sufficiently high, at least at about 2300° F.

Like a number of other chromium base alloys, it has been found that the alloy of the present invention can be further improved to resistance to oxidation and nitridation through the retention of yttrium and thorium such as in the range of about 0.05—0.2% Y and 0.05—0.2% Th. Below these amounts there is insufficient yttrium and thorium retained in the alloy either to getter the interstitials or to afford a significant amount of improvement in air oxidation resistance. Above those stated amounts, the alloy of the present invention tends to become embrittled.

One of the most useful forms of the alloy of the present invention is as a sheet material because of its high strength combined with good ductility and good air oxidation resistance particularly up to 1800° F. Because its processability is good, it is readily reduced into sheet from a cast form.

As was indicated above, the range of columbium included within the alloy of the present invention is 0.5—1.5 weight percent. The addition of amounts in excess of about 1.5% Cb allows the formation of too much CbCr<sub>2</sub> which is a coarse intermetallic phase. CbCr<sub>2</sub> tends to lower the melting point of the alloy and is detrimental to oxidation resistance. On the other hand, the inclusion of less than about 0.5 weight percent columbium in the presence of an excess of carbon allows the formation of the embrittling chromium carbide—such as Cr<sub>23</sub>C<sub>6</sub> rather than the fine columbium carbide. Thus the carbon range is controlled to be within the range of about 0.05—0.15 weight percent. The inclusion of too much of either columbium or carbon outside the range of the present invention leads to the formation of massive carbides. Unlike the fine carbide dispersion found in the present invention, the massive carbides lead to lower strength. In addition, the excess of columbium or carbon increases aging kinetics which has a significantly adverse effect on mechanical properties.

Typical of the alloys within the scope of the present invention are those listed in the following Table I in which compositions of the Cb/C atomic ratio is in the particularly beneficial range of 1—3 to 1.

TABLE I.—WT. PERCENT, BALANCE Cr

| Example | Zr    | Cb  | C    | Y    | Th   |
|---------|-------|-----|------|------|------|
| 1.....  | ..... | 1.0 | 0.11 | 0.06 | 0.11 |
| 2.....  | 0.21  | 1.1 | 0.11 | 0.08 | 0.12 |

A small amount of zirconium was added to the alloy of Example 2 because it was thought that the formation of zirconium carbide would stabilize columbium carbide. However, it was found that little if any zirconium was adsorbed by the columbium carbide phase as a result of

the early rejection of zirconium carbide by the chromium matrix upon solidification. Thus any stabilization of the columbium carbide through the use of zirconium is probably limited to the zirconium solubility in chromium. Therefore, the alloy of the present invention can include up to about 0.2 weight percent zirconium without significantly adverse effect on the mechanical properties of the alloy through the formation of the more massive zirconium carbide.

The alloy compositions shown in Table I were induction melted under argon to insure homogeneity and to minimize ingot cracking. The alloy was cast into a 3" diameter  $\text{Y}_2\text{O}_3$ -stabilized zirconia crucible. The yttrium and thorium additions in the charges were about 6 and 2 times, respectively, larger than the nominal contents to compensate for their losses through scavenging effects. Therefore the percentages for those elements listed in the specification refer to the retained amount rather than the amount added.

In order to provide sheet material for subsequent testing, the casting was extruded into bar before rolling into sheet. In order to effect carbide dissolution to allow control of dispersion either during extrusion or by post-extrusion heat treatment, higher extrusion temperatures were required. However, the extrusion temperature should not exceed 2800° F. to avoid incipient fusion. Therefore, a temperature of 2700° F. was selected for initial extrusion.

The extruded bar was first reduced 50% in thickness at about 2000° F. followed by rolling in the range of about 1500–1800° F. to produce the sheets of 0.05" thick material.

The rolled sheets were stress relieved at 2000° F. for 1 hour after which physical properties were determined.

The following Table II lists the tensile properties of the rolled sheet material in the stress relieved condition.

TABLE II.—TENSILE PROPERTIES  
[Rolled sheet, stress relieved (2,000° F./1 hr.)]

| Example | Temp.<br>(° F.) | Ultimate<br>Strength<br>(K s.i.) | 0.2% yield<br>strength<br>(K s.i.) | Elongation<br>(Percent) |
|---------|-----------------|----------------------------------|------------------------------------|-------------------------|
| 1-----  | 78              | 76.9                             | 67.0                               | -----                   |
|         | 500             | 70.1                             | 58.3                               | 10.4                    |
|         | 1,500           | 54.0                             | 49.2                               | 13.0                    |
|         | 1,800           | 42.9                             | 41.7                               | 12.0                    |
|         | 2,000           | 32.4                             | 27.4                               | 14.4                    |
|         | 2,200           | 18.6                             | 12.2                               | 32.8                    |
| 2-----  | 78              | 79.2                             | 49.8                               | 2.6                     |
|         | 500             | 58.9                             | 32.5                               | 7.0                     |
|         | 1,000           | 56.3                             | 28.6                               | 22.6                    |
|         | 1,500           | 49.9                             | 28.0                               | 25.2                    |
|         | 1,800           | 37.8                             | 27.8                               | 39.2                    |
|         | 2,000           | 28.6                             | 17.5                               | 63.6                    |
|         | 2,200           | 15.5                             | 12.9                               | 92.8                    |

A comparison between the alloy of the present invention and a known sheet alloy reported to be one of the best available based on chromium is shown in the drawing. The known alloy has a composition, by weight, of 93.5% chromium, 0.5% titanium and 6% magnesium oxide. Both sheet alloys were at the same thickness of

about 50 mils. The significantly better strength of the alloy of the present invention is shown by the drawing.

As was mentioned above, the alloy of the present invention is particularly suitable for use in an air oxidizing atmosphere. The good oxidation and nitrification resistance is shown by the data of Table III.

TABLE III.—100 HR. OXIDATION DATA

| Example | Temp., ° F. | Weight gain (mg./cm. <sup>2</sup> ) |           |
|---------|-------------|-------------------------------------|-----------|
|         |             | As cast                             | As rolled |
| 10      |             |                                     |           |
| 1       | 1,600       | 0.7                                 | 0.5       |
|         | 1,800       | 0.6                                 | 0.6       |
|         | 2,000       | 6.5                                 | 10.3      |
|         | 2,200       | 63.4                                | 60.7      |
| 2       | 1,600       | 0.6                                 | 0.6       |
|         | 1,800       | 1.1                                 | 0.9       |
| 15      |             |                                     |           |
|         | 2,000       | 13.7                                | 12.6      |
|         | 2,200       | 77.2                                | 69.4      |

Unlike alloys dispersion strengthened with more massive carbide such as zirconium carbide, the effect on oxidation resistance of reduction from cast to wrought condition is not great. The 100 hour oxidation tests conducted to obtain the data of Table III were performed on bar specimens of  $0.22 \times 0.35 \times 0.5''$  specimens in the rolled condition. The specimens were prepared by grinding and polishing through 400 grit paper followed by water and alcohol rinsing. Specimens were placed in zirconia crucibles and oxidized continuously in a tubular furnace with natural air convection.

Although the present invention has been described in connection with specific examples, it will be recognized by those skilled in the metallurgical art the modifications and variations of which the invention is capable and which are intended to be covered by the appended claims.

What is claimed is:

35 1. A chromium base alloy of improved strength consisting essentially of, by weight, 0.5-1.5% Cb; 0.05-0.15% C; 0.05-0.2% Y; 0.05-0.2% Th; up to about 0.2% Zr; with the balance chromium and incidental impurities.

40 2. A chromium base alloy of improved strength consisting essentially of, by weight, about 1% Cb; about 0.1% C; 0.05-0.2% Y; 0.05-0.2% Th; up to about 0.2% Zr; with the balance chromium and incidental impurities.

## References Cited

UNITED STATES PATENTS

|    |           |         |                      |        |
|----|-----------|---------|----------------------|--------|
| 50 | 2,955,937 | 10/1960 | McGurty et al. ----- | 75-176 |
|    | 3,011,889 | 12/1961 | Baranow -----        | 75-176 |
|    | 3,137,572 | 6/1964  | Aronin et al. -----  | 75-176 |
|    | 3,174,853 | 3/1965  | Sims et al. -----    | 75-176 |
|    | 3,208,847 | 9/1965  | Fox -----            | 75-176 |
|    | 3,227,548 | 1/1966  | Clark -----          | 75-176 |

## FOREIGN PATENTS

f 55 923.039 4/1963 Great Britain.

CHARLES N. LOVELL, *Primary Examiner.*